

1

2,847,292

## NITROFORM INHIBITED FUELS

Karl F. Hager, Clearfield, Pa., and Morris Rosenthal, Sherman Oaks, Calif.; said Hager assignor to the United States of America as represented by the Secretary of the Army

No Drawing. Application October 16, 1956  
Serial No. 616,354

14 Claims. (Cl. 52—5)

(Granted under Title 35, U. S. Code (1952), sec. 266)

The invention described herein may be manufactured and used by or for the Government for governmental purposes without the payment of any royalties thereon.

The present application is a continuation-in-part of our co-pending application, Serial No. 228,771, filed May 28, 1951. The latter application has become abandoned.

This invention relates to the protection of metals against corrosion.

Today aqueous solutions of alcohols, ketones and other water-soluble organic compounds are being utilized as propellants for rocket and other metallic internal combustion engines. Such propellants are well known to have a corrosive effect on iron and more particularly upon magnesium and other light metals. It is accordingly the main object of the invention to provide means for the protection of such metals from the corrosive action of propellant fuels and especially from the action of propellant fuels containing water.

To carry out the objects of this invention, the inventors have discovered that the addition of small amounts of nitroform or its salts to aqueous solutions of water-soluble organic fuels inhibits corrosive attack against metals. Nitroform is a colorless water-soluble explosive compound with a melting-point of 150° C. and the formula  $\text{CH}(\text{NO}_2)_3$ . Where this compound or one of its potassium salts is utilized, iron or steel containers are protected against corrosion from the aforementioned propellants. Magnesium containers, important in aviation and rocketry where weight must be kept to a minimum, are also protected and may be used with the aqueous propellants.

Illustrative of the practice of the present invention, the following examples are given:

## Example 1

Tests of the corrosion inhibition of nitroform were made by subjecting strips of mild steel about 40  $\text{cm}^2$  in area to inhibited and uninhibited water solutions of 75% ethanol contained in stoppered tubes at ambient temperatures. Similar tests were made by subjecting strips of mild steel about 40  $\text{cm}^2$  in area to inhibited and uninhibited water solutions of 50% acetone contained in stoppered tubes at ambient temperatures. The water-soluble organic compounds were inhibited with 0.05% of nitroform in different test tubes.

The mild steel pieces in the uninhibited fuels started rusting the first day and corroded more and more as time went on. The pieces in the inhibited fuels exhibited no corrosive effects for several months but after six months did show a few rust spots. Even after six months the surfaces remained 95% rustfree. By this time however the steel pieces in the uninhibited fuels were 100% covered by a thick layer of corroded metal and there was a heavy rust deposit at the bottom of each test tube.

2

## Example 2

The tests of Example 1 were repeated except for the substitution of magnesium strips for the steel strips.

The uninhibited fuels immediately showed an evolution of hydrogen bubbles caused by the corrosive attack on the magnesium. The inhibited fuels showed no trace of gas evolution while the magnesium in these fuels gave no evidence of corrosive attack. Within one month a white deposit of magnesium hydroxide had appeared in the bottoms of the test tubes containing the uninhibited fuels. No such precipitate was present in the test tubes containing the nitroform inhibited fuels. The surfaces of the magnesium in the uninhibited fuels had become totally encrusted with white crystals within six months. After six months magnesium in the inhibited fuels exhibited only a thin white crystalline deposit over a very small area. Excellent corrosion inhibition was obtained from the nitroform.

## Example 3

Samples of mild steel and magnesium were cut to give a surface area of approximately 37  $\text{cm}^2$  and were ground to a smooth surface. After degreasing, the samples were placed in individual test tubes and partially submerged in a water solution containing 75% ethanol. The potassium salt of nitroform was added to some of the test tubes of alcohol-water mixture in concentrations of 0.1% and 0.05% by weight. At the end of three days the samples were examined and the steel specimens placed in the alcohol-water mixture to which no inhibitor had been added had rust spots below and above the liquid-vapor interface. The magnesium specimens in the uninhibited alcohol had large discolored areas indicating corrosion in the liquid portion of the system although the portion in the vapor seemed not to be affected. The specimens of steel and magnesium in the alcohol-water mixture inhibited by the potassium salt of nitroform showed very little, if any, corrosion. It should be noted that the inventors do not wish to be limited by any theory for the disassociation of the potassium salt or salts while in solution.

## Example 4

Samples of steel and magnesium were cut, conditioned, and tested in the same manner as in Example 3. However, the samples were partially emerged in a water solution containing 50% acetone. The potassium salt of nitroform was added in concentrations of 0.1% and 0.05% by weight. In a three day period discolored spots were evident on the steel and magnesium samples in the uninhibited fuel. The steel and magnesium samples which were in the acetone-water mixture inhibited with 0.1% and 0.05% potassium salt showed very little, if any, corrosion.

We claim:

1. A liquid fuel mixture consisting essentially of a major amount of an aqueous solution of a water soluble organic compound of the class consisting of alcohols and ketones and a minor amount of an inhibitor of the class consisting of nitroform and the potassium salts of nitroform sufficient to inhibit corrosion of metal surfaces.
2. A liquid fuel consisting essentially of a mixture of water and an organic compound of the class consisting of water soluble alcohols and ketones and a minor amount of nitroform sufficient to inhibit corrosion of metal surfaces.
3. A liquid fuel consisting essentially of a mixture of water and an organic compound of the class consisting of water soluble alcohols and ketones and a minor amount

of the potassium salts of nitroform sufficient to inhibit corrosion of metal surfaces.

4. The method of protecting metal surfaces of the class consisting of iron, steel and magnesium from the corrosive action produced by liquid fuel mixtures consisting essentially of water and a water soluble organic compound of the class consisting of alcohols and ketones in contact therewith, which comprises contacting said fuel mixture with the metal surface in the presence of a small amount of an inhibitor of the class consisting of nitroform and the potassium salts of nitroform sufficient to inhibit corrosion, and thereby treating said metal surfaces to produce a corrosion inhibiting action thereon whereby said surfaces are rendered substantially inactive with respect to the normal corrosive action of said fuel mixtures.

5. The method of protecting metal surfaces of the class consisting of iron, steel and magnesium from the corrosive action produced by liquid fuel mixtures consisting essentially of water and a water soluble organic compound of the class consisting of alcohols and ketones in contact therewith, which comprises contacting said fuel mixture with the metal surface in the presence of a small amount of nitroform sufficient to inhibit corrosion, and thereby treating said metal surfaces to produce a corrosion inhibiting action thereon whereby said surfaces are rendered substantially inactive with respect to the normal corrosive action of said fuel mixtures.

6. The method of protecting metal surfaces of the class consisting of iron, steel and magnesium from the corrosive action produced by liquid fuel mixtures consisting essentially of water and a water soluble organic compound of the class consisting of alcohols and ketones in contact therewith, which comprises contacting said fuel mixture with the metal surface in the presence of a small amount of the potassium salts of nitroform sufficient to inhibit corrosion, and thereby treating said metal surfaces to produce a corrosion inhibiting action thereon whereby said surfaces are rendered substantially inactive with respect to the normal corrosive action of said fuel mixtures.

7. A liquid fuel consisting essentially of 75% ethanol, and water, to which has been added approximately 0.05% nitroform as a corrosion inhibiting agent.

8. A liquid fuel consisting essentially of 75% ethanol, and water, to which has been added from between 0.05% to 0.1% of the potassium salts of nitroform as a corrosion inhibiting agent.

9. A liquid fuel consisting essentially of 50% acetone,

and water, to which has been added approximately 0.05% nitroform as a corrosion inhibiting agent.

10. A liquid fuel consisting essentially of 50% acetone, and water, to which has been added from between 0.05% to 0.1% of the potassium salts of nitroform as a corrosion inhibiting agent.

11. The method of protecting metal surfaces of the class consisting of iron, steel and magnesium from the corrosive action produced by a liquid fuel mixture consisting essentially of 75% ethanol, and water, which consists in adding to said fuel mixtures about 0.05% nitroform, and thereby treating said metal surfaces with said nitroform as an agent to produce a corrosion inhibiting action on said metal surfaces, whereby said surfaces are rendered substantially inactive with respect to the normal corrosive action of said fuel mixture.

12. The method of protecting metal surfaces of the class consisting of iron, steel and magnesium from the corrosive action produced by a liquid fuel mixture consisting essentially of 75% ethanol, and water, which consists in adding to said fuel mixture from between 0.05% to 0.1% of the potassium salts of nitroform, and thereby treating said metal surfaces with said potassium salts of nitroform as an agent to produce a corrosion inhibiting action on said metal surfaces, whereby said surfaces are rendered substantially inactive with respect to the normal corrosive action of said fuel mixture.

13. The method of protecting metal surfaces of the class consisting of iron, steel and magnesium from the corrosive action produced by a liquid fuel mixture consisting essentially of 50% acetone, and water, which consists in adding to said fuel mixture about 0.05% nitroform, and thereby treating said metal surfaces with said nitroform as an agent to produce a corrosion inhibiting action on said metal surfaces, whereby said surfaces are rendered substantially inactive with respect to the normal corrosive action of said fuel mixture.

14. The method of protecting metal surfaces of the class consisting of iron, steel and magnesium from the corrosive action produced by a liquid fuel mixture consisting essentially of 50% acetone, and water, which consists in adding to said fuel mixture from between 0.05% to 0.1% of the potassium salts of nitroform, and thereby treating said metal surfaces with said potassium salts of nitroform as an agent to produce a corrosion inhibiting action on said metal surfaces, whereby said surfaces are rendered substantially inactive with respect to the normal corrosive action of said fuel mixture.

No references cited.